

# United States Patent Office

2,930,756

Patented Mar. 29, 1960

1

2,930,756

## COMPOSITION FOR SCALE CONDITIONING AND LUBRICATION OF METALS

Robert A. Simon, Seattle, Wash., assignor to North American Aviation, Inc.

No Drawing. Application May 27, 1955  
Serial No. 511,745

1 Claim. (Cl. 252—25)

This invention pertains to a metal conditioning composition and more particularly to a composition which conditions scale on titanium and stainless steel for subsequent removal, and which is additionally an effective metal working lubricant.

With the advent of titanium and its alloys as production metals numerous problems have resulted from a metal working standpoint. One of the difficulties results from the formation of a complex scale on the surface of titanium metal and its alloys when it has been subjected to heat such as in forming, heat treating or the like. This scale not only gives a poor appearance but it also interferes with inspection procedures, lessens the ductility of the metal and can interfere with welding. Removal of this scale therefore becomes imperative. It has been past practice to use an acid pickling bath to remove the scale after the parts have been subjected to heat. This was a passable solution to the problem while forming and heat treating of titanium remained at relatively low temperatures. However, now titanium parts are being subjected to temperatures up to 1100° F. and a heavier scale is formed of such character that all known acid pickles have proved to be unsatisfactory. In the first place where a part has been given a scale at a relatively high temperature it is necessary to leave it in the pickle for a considerable period of time which becomes a severe penalty from a production stand-point. Also, the active ingredients in the bath are rapidly depleted. Even more important, in removing scale in this manner an excessive amount of metal will be lost so that it becomes impossible to keep the work piece within prescribed tolerances. As much as 10 percent of the thickness of light gauge parts may be lost in descaling. Furthermore, the scale removal will be imperfect over the surface of the part, considerably more scale being removed from some portions than others.

A similar problem has been encountered with the use of 17-7 PH stainless steel. This is a precipitation hardening stainless steel containing around 17% chromium, 7% nickel, and 1% aluminum more fully described in Military Specification MIL-S-25043 (ASG). This material may be heated in a typical heat treat cycle to 1900° F. for annealing and cured at 1400° F. which provides a severe scale condition on the surface of the part comprising a magnetic iron oxide material having  $Fe_3O_4$  in a high proportion. This is a very stable scale which is not attacked by an ordinary acid bath. It has been attempted to remove the scale by abrasives, but this too has difficulties not only from the practical standpoint of covering the entire area, but also from the degree of surface roughness which the abrasives cause. In one instance it was desired to resistance weld a 17-7 PH stainless steel part from which the scale had been removed by an abrasive process. The roughness resulting from this descaling procedure was so great that resistance welding became impractical because a uniform contact could not be obtained.

The metal bath of this invention is applied to the

2

titanium or 17-7 PH stainless steel workpiece prior to its heating and causes the scale formation to be of such character that it can be removed by existing acid baths with relative ease and reliability.

5 A metal working lubricant obviously must possess the basic qualities which enable it to so protect the part and die during a forming operation so that there is no damage to either. For this purpose it must be adherent and tough. Also it should be simple to handle and apply, and preferably can be applied to the part prior to its 10 introduction into the area of a press where the part was to be formed. This will keep the press area clear and allow the lubricant to be applied in a more orderly manner. Ideally the material used as a lubricant should also 15 form a durable coat which will protect the part during its handling. Removal is the next major problem, which for metal working lubricants generally involves scrubbing with suitable solvents. The bath of this invention provides a metal working lubricant which answers all 20 of these requirements. It is not only extremely effective for room temperature forming operations but provides a tough protective film which may be applied long before the part is formed. Removal of the lubricant involves only dipping of the part in water whereupon it will all 25 be dissolved and the part will be clean.

Accordingly, it is an object of this invention to provide a material which will condition scale formations so as to permit subsequent complete scale removal from a short dip in a conventional acid pickle bath. Additionally, it is an object of this invention to provide a conditioning material which is easily applied and removed, and gives protection to a workpiece during handling. A further object of this invention is to provide a material effective as a metal working lubricant which will protect 30 part and die during a forming operation. Yet another object of this invention is to provide a single material serving the functions of part protection, lubrication for forming, and conditioning for scale formations obtained when the part is heated. These and other objects will 35 become apparent from the following detailed description.

40 Considering first the problem of a pretreatment for minimizing scale and permitting it to be readily removed subsequent to heating, I have found that basically the 45 results may be obtained by applying borate or a boron bearing material to the titanium or 17-7 PH stainless steel prior to its being subjected to high temperature. This will so condition the scale which is formed so that it can be removed without difficulty. No problem of 50 hydrogen absorption is encountered with the compound of this invention.

A particular composition which has proven to be successful is as follows:

| Component:                        | Percent by weight |
|-----------------------------------|-------------------|
| 55 Boric acid, tech.              | 7.8 to 8.2        |
| Shellac, orange flake             | 4.0 to 4.5        |
| Diethylamine, tech.               | 3.3 to 3.5        |
| Dye                               | .05 to .06        |
| 60 Water, distilled or de-ionized | 4.0 to 5.0        |
| Methanol, Federal Spec. O—M—232   | Remainder         |

65 The boric acid contained in the substance of the above description is the primary material which serves to modify the scale formation. It can be operatively used alone, but from the standpoint of application, adherence and handling this is, of course, not a practical matter for a pretreatment compound to be used in production. Boric oxide, if substituted in the above compound, will hydrolyze into boric acid and therefore may replace that ingredient. Boron bearing materials containing potassium and sodium have been found to be harmful to titanium

when it is subsequently subjected to heat. Consequently they should not be used in a pretreatment compound.

The shellac is included primarily to serve as a binder. For this purpose alone it might be satisfactory to use another type of binder such as, for example, varnish. However, shellac is chosen because it has some effect of its own in modifying the scale formation so as to permit the subsequent removal thereof.

The ammonia carrying compound, diethylamine, is mainly to give the solution water solubility. Ammonium hydroxide may be used in lieu of the diethylamine, but results in a material not quite as stable as when the latter substance is included. Ethylene diamine may also be substituted for diethylamine. The ammonium carrying material used should have a relatively low boiling point and be a strong base readily yielding its ammonia radical. Heavier materials will become gummy rather than properly drying out. Other bases such as sodium, potassium and calcium hydroxides actually have a harmful effect on the metal and cause spots which cannot later be pickled off.

The primary purpose of the methanol is to act as a solvent. The water in the solution serves to hydrolyze the methyl borate that is formed with the boric acid, preventing its loss. Therefore, when the composition is prepared it is important to combine the water and methanol before adding the boric acid. Because sodium or potassium salts have a deleterious effect on titanium when subsequently heated, it is necessary to use distilled or deionized water.

Ethanol may be employed in the composition as a substitute for the methanol with no loss in desirable characteristics. The use of ethanol avoids the toxicity which is present when methanol is used. Commercial ethanol contains around five percent water, so further addition of water to the composition is unnecessary when this material is used. Isopropanol is also acceptable. Heavier alcohols, however, have a greater drying time and for that reason are not as desirable for use in the compound. The main advantage of methanol is that more boric acid will go into solution therein than into these other alcohols.

The dye in the composition serves merely as an indicator giving the compound enough color so that it is possible to determine exactly what portions of the part have been covered. Any suitable alcohol soluble dye may be used.

The material so prepared may be applied in any desired manner such as brushing, dipping or spraying, with the latter generally proving more convenient. The result is a coating which is adherent and tough so that the part receives protection prior to the heat treating operation, and which also assures that there is little likelihood of losing the coating from the surface of the part.

As far as the proportions indicated for the solution are concerned some variation may be permitted, but the range indicated represents what is believed to be an optimum condition for the ingredients included. The acid, being the primary agent for conditioning the scale which is formed, is of course desirable in relatively large amounts. However, if too much of this material is included it will not go in solution so the range indicated cannot be exceeded by very much. Although the shellac is an excellent binder and has its own effect in scale conditioning too much of this ingredient can result in carbon deposits on the surface of the metal, if it is later subjected to heat, as the shellac burns. Some of these spots can become so severe that removal is impossible. In order to provide proper saponification for the composition diethylamine should be included approximately as indicated. Above this range no additional benefit is obtained although it is possible to include up to about 10 percent by weight without harmful effect.

This composition, when applied to the surface of a workpiece, has in addition to its scale deterrent characteristics the ability to act as an extremely effective dry

forming lubricant for metal working, which use may even prove to be more important than that of treating the metal for scale formation. The material provides a very slippery surface for the workpiece while at the same time adhering very tenaciously, and will hold on even when drawn or pulled into a die. As the part is being formed it appears to provide a cushioning effect which protects the metal and die and permits the forming to take place. The minute quantity of the material which will be rubbed off as the metal is formed builds up slightly on the die surface thus providing a polishing effect and a more smooth and effective die is obtained. For its use as a lubricant it is preferred to spray on two coats of the material prior to the forming operation so as to provide a relatively thick coat on the part. After the forming operation the material may be left on for further heat treat or other work whereby a dual function can be obtained from the material. First it will act as a lubricant in permitting forming of the part, and secondly will retard scale formation and condition the scale when the part is subsequently heat treated. However, if it is desired to remove the material immediately after the metal forming this is quite easily accomplished due to the water solubility thereof. Mere dipping in water will thoroughly cleanse the part without scrubbing. Although it has primarily been used for a cold forming lubricant it is also useful in hot forming where it acts as a base for an additional conventional lubricant coating applied at the time the hot forming is to take place. Results for both types of forming are materially improved when the metal surface is coated. Its use as a forming lubricant is applicable not only to titanium and 17-7 PH stainless steel but also to other steels, aluminum and other metals as well.

Several advantages therefore may be listed for the material as a metal forming lubricant. First and foremost it produces superior parts and considerably increases die life. The fact that it can be applied before the time of forming is an advantage in production and provides a protection of the part during material handling. Application of the lubricant by spraying means that there is no waste of material and cost is much lower than with ordinary lubricants. Furthermore the lubricant may be retained on the surface part for subsequent heat treating or, if desired, it may be removed simply by dipping in water.

A second formulation of the composition of this invention has been successfully carried out and also is quite effective in pretreatment for scale formations as well as a metal lubricant. For the latter purpose, it is primarily for instances where the part will be subsequently subjected to heat to avoid a removal problem. This solution is as follows:

| Component:                                              | Percent by weight |
|---------------------------------------------------------|-------------------|
| Boric acid, tech.                                       | 3.5 to 4          |
| Shellac, orange, four pound cut, Federal Spec. TT-V-91B | 33 to 50          |
| Dye                                                     | .05 to 1.0        |
| Ethyl alcohol, Federal Spec. O-A-396                    | Balance           |

It may be noted that the compound in the second example contains no amine as it is shown. This has one advantage where parts are to be treated and stored for some time prior to their working or heat treatment. Without the amine the compound is not water soluble and the moisture in the air will not attack the solution so that the coating will remain on the part indefinitely. However, if it is desired to provide a water soluble solution, around one percent of an amine added to the above formulation will provide this effect. Note that the use of ethyl alcohol means that ethyl borate will be formed when the compound is made up, this being a non-volatile liquid. Therefore, there is no problem of loss of the borate as encountered with gaseous methyl borate. The proportions of the ingredients should be retained substantially as indicated in the table; boric acid above for percent in the solution causes it to be somewhat unstable and reduces

its shelf life. The larger quantity of shellac used with this modification will suspend any particles of boric acid that have not gone into solution to assure that an adherent coating is obtained.

Another variation of this compound has been prepared and shown to provide utility in retarding scale formations, but it is not regarded as quite as effective as the previously given examples. This modification comprises one part of boric acid suspended in a solution of one part shellac, four parts of methanol and one part isopropanol.

It can be seen from the foregoing that I have provided an improved metal treating material which has numerous advantages for both of its dual functions. Scale formations for titanium and 17-7 PH stainless steel are greatly reduced while the material offers tremendous advantages as a dry lubricant for metal forming.

The foregoing detailed description is to be regarded as given by way of example only, the spirit and scope of this invention being limited only by the appended claim.

I claim:

A metal treating composition consisting of a solution

of substantially 7.8 to 8.2 percent by weight boric acid, 4.0 to 4.5 percent flake shellac, 3.3 to 3.5 percent diethylamine, 4.0 to 5.0 percent water, and the balance of a material taken from the group consisting of ethanol, methanol and isopropanol.

References Cited in the file of this patent

UNITED STATES PATENTS

|    |           |           |                |
|----|-----------|-----------|----------------|
| 10 | 1,896,040 | Ruben     | Jan. 31, 1933  |
|    | 1,923,058 | Lawstuter | Aug. 15, 1933  |
|    | 2,483,598 | Schrank   | Oct. 4, 1949   |
|    | 2,588,234 | Hendricks | Mar. 4, 1952   |
|    | 2,762,115 | Gates     | Sept. 11, 1956 |

FOREIGN PATENTS

|    |         |               |                |
|----|---------|---------------|----------------|
| 15 | 151,688 | Great Britain | Sept. 20, 1920 |
|----|---------|---------------|----------------|

OTHER REFERENCES

|    |                                                                   |
|----|-------------------------------------------------------------------|
| 20 | Bastian: "Metal Working Lubricant," McGraw Pub. Co., 1951, p. 19. |
|----|-------------------------------------------------------------------|